

Mar. 3, 1925.

1,528,407

S. A. DAVIS

MANUFACTURE OF TIN PLATE

Filed June 25, 1919

3 Sheets-Sheet 1



FIG. 1

INVENTOR  
S. A. Davis  
by Anthony Uanna  
his Attorney

Mar. 3, 1925.

1,528,407

S. A. DAVIS

MANUFACTURE OF TIN PLATE

Filed June 25, 1919

3 Sheets-Sheet 2

FIG. 2



INVENTOR

*S. A. Davis  
by D. Anthony Neira  
his Attorney*

Mar. 3, 1925.

1,528,407

S. A. DAVIS

MANUFACTURE OF TIN PLATE

Filed June 25, 1919

3 Sheets-Sheet 3



FIG. 3



FIG. 5

INVENTOR

by S. A. Davis  
D. Anthony Neiva  
his Attorney

## UNITED STATES PATENT OFFICE.

STEWART A. DAVIS, OF PITTSBURGH, PENNSYLVANIA, ASSIGNOR TO AMERICAN SHEET AND TIN PLATE COMPANY, OF PITTSBURGH, PENNSYLVANIA, A CORPORATION OF NEW JERSEY.

## MANUFACTURE OF TIN PLATE.

Application filed June 25, 1919. Serial No. 306,521.

To all whom it may concern:

Be it known that I, STEWART A. DAVIS, of Pittsburgh, in the county of Allegheny and State of Pennsylvania, have invented 5 certain new and useful Improvements in the Manufacture of Tin Plate, of which the following is a specification.

My invention relates generally to the manufacture of tin plate. The invention 10 more particularly relates to the manufacture of that cheaper grade of tin plate having a relatively thin or light weight coating of tin known commercially as "coke plate".

Tin plate is sold universally by the base 15 box, a base box being the equivalent of 112 plates, 14 inches by 20 inches by 30 gage, or totalling 31360 square inches superficial area.

The standard commercial grade of "coke 20 plate" carries approximately one and one-half pounds of tin per base box, is without a high lustre, and is dull or dry in appearance. The coating on commercial coke plate is not entirely continuous, but contains small 25 openings or channels running through the coating to the ferrous sheet underneath and forming what is technically known as "pin holes". As the thickness of the tin coating is increased on commercial coke plate its 30 lustre is improved, approximately in proportion as the weight of tin per base box increases. The number of pin holes, however, do not decrease in this same proportion. Thus a coke plate carrying two pounds of 35 tin per base box has a distinctly higher lustre than a plate coated with one and one-half pounds, although the number of pin holes per unit of area is not materially changed.

40 The process of manufacturing tin plate, as carried on heretofore, consists essentially in passing the cleaned iron or steel plate or base, by hand, through a layer of flux into a bath of molten tin, subsequently with- 45 drawing the plate and removing the sur- plus adhering tin from the surface by means of rotary, spring pressed sets of exit rolls. When the ferrous base and molten tin first come into contact, a layer of an iron-tin 50 alloy forms on the surfaces of the base, this alloy having a melting point higher than that of the molten tin itself. The re- 55 sult of this action is that fine needle-like crystals of this iron-tin alloy are formed

which protrude from the surfaces of the 55 iron base and form a fine spongy or porous network of crystals, the interstices of which are filled with the molten tin. When the iron base and adherent alloy layer of crystals later pass between the exit rolls of the tin- 60 pot, which are located within a body of palm oil, the network of crystals is crushed and flattened against the iron base, and a large portion of the molten, interstitial tin 65 is squeezed out and flows off the plate. The body of molten tin within the pot in reality soon becomes a saturated solution of iron-tin alloy in molten tin, this being shown by the large amount of scruff or iron-tin 70 alloy which becomes deposited on the bottom 75 of the pot, in the oil or exit end of the pot.

The plate, as it emerges from between the exit rolls, therefore, consists of the ferrous base covered with a coating which is composed of a mixture of the crystals of iron-tin alloy and pure tin. The presence of the 80 crystals produces what can be seen under a microscope to be a rough irregular surface, which in turn imparts the dull or as technically termed, the "dry" appearance of 85 the surfaces of the coke plate.

In carrying out the old process great care is taken to keep the "yield" at or below a certain limit, the yield varying with different 85 grades of tin plate and being determined by the particular grade of tin plate being made. The yield has been controlled by regulating the speed at which the plates are fed out of the tin-pot, the general practice being to reduce the speed of feeding the 90 plates through the tinning machine (within certain limits) to lessen the yield. This was done because experience had shown an increase in the speed of passing the plates through the tinning bath was followed by 95 an increase in yield. A speed of from 100 to 120 inches per minute has been considered the maximum possible in making coke plate. It also is a matter of general knowledge that keeping the plates within the bath of molten tin for too long time interval results in 100 making plates having black spots (i. e. spots where the tin does not adhere to the base).

The primary object of my invention is 105 the provision of a novel method of applying the coating of tin to the iron or steel plates whereby the speed at which the tinning operation is effected can be very materially

increased without undue increase in the "yield", (a trade term denoting the amount of tin used in coating per unit of area of the coated surfaces,) and whereby the capacity of the tinning machines is greatly increased and the cost of making tin plate correspondingly lessened.

Another object of the invention is to provide an improved method of tinning ferrous metal plates whereby, without increase in the yield, a product is obtained having the very high lustre characteristic of the heavily coated, high grade tin plate, such as "charcoal plate", and the absence of pin holes characteristic of both coke and charcoal grades as heretofore made by the old process.

Another object of the invention is to provide an improved method of making coke plate whereby the yield or weight of tin per unit of area of the coke plate may be materially reduced, and an enormous saving in the amount of tin used is thereby effected, with a correspondingly great reduction in the cost of production.

Another object of the invention is the production of a new article of manufacture, viz,—a coke plate which combines the lustrious appearance characterizing the heavily coated tin plate such as charcoal plate with the thin or light weight coating which distinguishes ordinary coke plate.

Another object of the invention is the production of tin plate in which the pin holes and other imperfections present when made by the old process are lessened and overcome.

Referring now to the drawings forming part of this specification, Figure 1 is a plan showing a tinning pot constructed and arranged in accordance with this invention.

Figure 2 is a longitudinal section, on the line II—II of Figure 1, showing a preferred arrangement of apparatus embodying the invention and adapted for use in carrying out the method forming part of my invention.

Figure 3 is a sectional end elevation, on the line III—III of Figure 2, showing further details in the construction and arrangement of the apparatus.

Figure 4 is a plan, and Figure 5 is a side elevation showing details in the construction of the roll and feed roller driving mechanism forming part of my improved tinning machine.

In the accompanying drawings, the letter A designates a tinning pot, in itself an old and approved form. The pot is separated transversely by a vertical wall or partition 2 into compartments B and C. The lower edge of this septum 2, which terminates above the bottom of the tinning pot, and the upper edge of a rib or projection 3 on the bottom of the pot defines the width or ver-

tical dimensions of a narrow passage or opening D through which the plates, while submerged in the bath of molten tin, pass from the compartment B into the compartment C of the pot A. The particular pot shown is of a width which permits of two or more plates, side by side, being passed through the tinning pot. (See Figures 1 and 3.) Obviously, when desired, a narrower pot of a width slightly greater than the width of the widest plate may be used. Any of several known means may be provided for heating the tinning pot and preferably these means will be constructed and arranged to maintain the tin in the compartment B at a considerably higher temperature than the molten tin in the compartment C.

The heating apparatus, not forming part of this invention, is not shown nor further described.

The side walls of the compartment C at the exit end of the pot are extended upwardly so that this compartment is considerably deeper than the other compartment B, this old and well known construction enabling a body of oil, generally palm oil, of the requisite depth or thickness, to be maintained on top of the molten tin in the compartment C. The levels at which the bath of molten tin is maintained in the pot are indicated by the line X—X of Figure 2, and a thin layer H of flux, such as zinc chloride, is maintained on top of the tin in the compartment B on the entrance end of the pot. It is due to the weight of this body of oil that the level of the tin bath in the compartment C is somewhat lower than that of the molten bath in the compartment B. The upper level at which the oil is maintained in the compartment C is indicated by the line Z—Z.

Located immediately above the upper edge of the compartment B, at the plate entering side of the tinning pot, are two sets of spring pressed feed rollers E and F, which are arranged to move the pickled and washed plates forwardly and downwardly into the tin-pot at an angle to the horizontal. The rollers 6 and 7 forming the set F are at a somewhat lower level than the rollers 4 and 5 of the set E. An adjustable roller G, located on the discharge side of the set F, is provided to guide and direct the front end of the successive plates forwardly and downwardly through the layer of flux H into the molten tin in compartment B, as they emerge from between the rollers of the set F.

Positioned within the compartment B, closely adjacent to the passage D, is a set of pressure rolls I. These pressure rolls, which are submerged in the molten tin, have the double function of feeding the plates from the compartment B into the compartment C

of the tinning pot, and they also are arranged to be rigidly held in close engagement so as to not only feed the plates forwardly, but also to flatten and smooth the 5 layer of iron-tin alloy which is formed on the iron or steel plates or sheets as the plates enter the molten tin in compartment B of the tin-pot. This flattening and smoothing operation by the rolls 8 and 9 of the set I is 10 novel, and forms a vital and very important part of my invention, as will be more fully explained hereinafter.

It should be noted that the sets of feed-in rollers E and F and the guide roller G 15 are above the layer of flux H, and that the successive plates are mechanically fed and guided into the tinning pot.

The location of the pressure rolls I with respect to the layer of flux H also should be 20 noted. It has heretofore been considered impossible to use submerged feed-out rollers in a tinning machine. This is because experience shows that long contact of the rolls with the molten tin bath causes the layer of 25 tin on the rollers to flake off and bare the surface of the rollers, and that when this occurs the result is the making of defectively coated plates, known in the art as having "black spots" i. e.—plates having uncoated spots on the surfaces thereof.

But by positioning the pressure rolls I so that the distance from the flux H is not too great, sufficient flux is carried down by the plates to maintain the rolls I in working 35 condition.

Two sets of feed-out rollers J and K are provided which are located within the body of oil maintained on top of the tin in the compartment C of the pot A. The sets of 40 rollers J and K are arranged to not only feed the plates out of the tin-pot, but also act to squeeze off surplus tin from the smooth alloy coated surfaces of the plates passing upwardly out of the tinning pot. The body of oil 45 in which these rollers are submerged acts to prevent the molten coating on the surfaces of the plates from contacting with the atmosphere, until after the excess coating has been removed therefrom.

An inclined apron plate 14 is provided at 50 the entrance end of the compartment B of the pot to receive the plates as delivered to the tinning pot. Plates 15 and 16 form a guide L for directing the front end of the successive plates as they merge from between the set of rollers E into the bite of the set F.

Curved guide plates 17 and 18 forming a 55 guide M are positioned within the compartment B so as to direct the forward end of the plates being tinned into the nip of the set I of pressure rolls, as is clearly shown in Figure 2. These guide plates 17, 18, preferably, are made of skeleton form so as to 60 not interfere with the settling of scruff and

any foreign material in the molten tin to the bottom of the compartment B of the pot.

Curved guide plates 19 and 20 form a 70 guide N which directs the forward end of the plates emerging from the set of pressure rolls I upwardly into the bite of the lower set J of two sets of feed-out rollers J and K within the upper end of the compartment C of the tin-pot. It will be seen by 75 reference to Figure 2 that the rear end of the curved lowermost guide plate 20 extends backwardly through the passage D into proximity to the set of rolls I.

The frame work O, which supports the 80 sets of feed rollers E and F, guide roller G and pressure rolls I and the stationary guides L and M, is removably secured within the compartment B so as to permit of the feed-in apparatus to be removed bodily from 85 the pot while the tin bath is molten. This is done at intervals in order to clean the tinning pot, and when necessary to make repairs to the feed-in apparatus. The sets of feed-out rollers J and K and guide N are 90 similarly mounted on a frame work P in the compartment C of the pot, and are taken out of and replaced in the compartment C in the same manner as the apparatus within the 95 other compartment B.

The feed rollers 4 and 5 of the set E are connected together by pairs of spur gears 21 to positively drive these rollers at the same surface speed, and the rollers 6 and 7 of the set F have meshing spur gears 22 on one 100 end for a similar purpose. The rolls 8 and 9 also have meshing spur gears 23 on one end to positively rotate these rolls.

The pairs of feed-out rolls forming the 105 sets J and K in the compartment C of the tinning pot also are geared together by spur gears 24 to positively rotate the pair of rolls forming each set.

The rolls 8 of the pressure rolls and the 110 rollers 6 and 4 of the sets of feed-in rollers F and E are connected together by bevel gears 25, one gear of each pair being keyed on the shaft 26 and this shaft being rotatably secured in bearings 27 mounted on an angle support 28 which is fastened on one 115 side of the frame work O in the compartment B.

A spur gear 29 on the end of the feed 120 roller 4 meshes with a similar gear 30 on the stub shaft 31 and this stub shaft has a sprocket wheel 32 on one end which is driven by a sprocket chain from a suitable motor (not shown).

The rollers forming the sets of feed-out 125 rollers J and K are positively driven in the usual and well known manner.

In carrying out my improved process with a tinning machine constructed essentially as shown and described, the plate or sheet of iron or steel, after being pickled and 130

washed, is placed on the apron 14 and is moved downwardly thereon until its front end enters the nip of the set E of feed rollers. The plate, upon emerging from between these rollers passes through the guide L into the nip of the second pair F of feed rollers, which are located immediately above the layer of flux H in the flux box.

The plates as supplied to the apron 14 from the washing bath have some water adhering to them. The wet plates in passing through the feed rollers E and F are freed from substantially all water, the small amount remaining acting to maintain the flux in a suitable condition. With the displacement of this excess water there also is removed from the plates certain foreign materials which frequently adhere thereto.

In passing from between the rollers F, the plate is directed into the flux H by the adjustable guide roller G so that the plate at no time comes into contact with any extension or guide projecting below or beyond the level of the flux. This provision of means for entering the sheets into the tin through the flux without having the plates come in contact with any stationary part of the pot avoids the dislodgement of congealed flux and other substances which have previously been deposited and which would otherwise be carried into the molten tin bath. The rapid downward movement of the sheet through the flux into the tin bath and between the pressure rolls I carries sufficient flux to these submerged rolls to maintain them in proper working condition.

After passing through the flux, the plate enters the molten tin in the compartment B, passing through the curved guide M. This guide is preferably of skeleton construction as shown, so as to permit the deposition of scruff or other foreign materials on the bottom of the compartment B. The guide M discharges the plates into the nip of the set of pressure and cleaning rolls I which are preferably made from solid steel and are ground and polished. The rolls I, obviously, will be provided with a suitable mechanism for regulating the pressure on the plates passing between them, and as has been stated, will be driven by a mechanism which provides a uniform lineal speed for the sheet as it passes through the pot.

In passing the plates between the pressure rolls I, the porous mass of needle-like crystals of iron-tin alloy formed on the plate as it passes into the molten tin bath, is rolled down and flattened and smoothed, and the surplus, interstitial tin, which is still molten, is squeezed out and removed from the alloy coating now on the plate. Some tin alloy coating also is removed, as is shown by the deposit of scruff which collects on the bottom of the pot below these rolls. From the rolls I, the plate, now hav-

ing a flattened and smoothed iron-tin alloy coating, passes through the opening D and is deflected by the curved guide N into the nip of the first pair of feed-out rollers J, and thence between the second set K, and 70 out of the tinning pot.

The iron-tin alloy, formed as a porous, spongy net-work of very fine crystals upon the iron sheet, when the plate enters the tin bath, is flattened out and pressed closely 75 upon the plate by the rolls I. There being but little agitation of the molten metal in the pot, the flattening and smoothing operation and the removal of the excess iron-tin alloy while the plate is in the compartment 80 B and before reaching the compartment C of the tin-pot, the tin in the compartment C remains substantially pure and does not become saturated with iron-tin alloy as with the old methods. Any excess alloy not 85 tightly adhering to the sheet also is removed and is forced into the tin bath, finally settling to the bottom of the pot directly below the rolls. This disposition of the rolls I relative to the slot or passage D in the 90 pot prevents contamination of the tin on the oil side of the slot by the accumulated scruff or alloy and other impurities which, in the present case, collect in the pot in the flux side of the passage D and become deposited 95 in the compartment B.

Any excess tin adhering to the smoothed and flattened iron-tin alloy on the plates is removed by the pressure of the sets of feed-out rollers J and K, and a finished coke 100 plate is provided having an outer layer of substantially pure tin which has the lustre and other properties characteristic of the heavier coating of charcoal plates.

The most important advantage of my invention, as will be appreciated by those skilled in the art, arises from the very considerably increased speed at which the plates can be passed through the tinning machine without increase in the "yield", and in 110 many cases with an actual decrease in the "yield".

Another advantage is that instead of feeding the plates through the pot at a speed of not exceeding about 120 inches per minute, they can travel at a rate up to 200 or more inches per minute, and this increased speed results in an enormous increase in the capacity of the tinning pots, while the action of the pressure rolls results 120 in a large saving in the amount of tin used for coating the plates. The increased speed of tinning and reduction in yield is made possible through the removal of excess tin from the interstices of the spongy, porous 125 layer of iron-tin alloy (which is formed on the plates as they enter the bath of molten tin), by the considerable pressure exerted by the pressure rolls and the flattening and smoothing of the alloy layer, at a time early 130

enough in the tinning operation for the flattened and smoothed coating of alloy to acquire a second coating of substantially pure tin and early enough for any excess tin to be wiped off or removed from the alloy coating by the action of the feed-out rollers, instead of having the spongy, porous alloy layer acted upon only by the feed-out rollers, as is the case in the methods used heretofore.

10 A further advantage is in the production of a superior coke plate having the finish or lustre of the heavily coated charcoal plates and having a lighter coating of tin than is possible with any known process or apparatus heretofore used in making coke or other tin plate.

Modifications in the construction and arrangement of the apparatus used in carrying out the method forming part of this invention may be made without departing from the invention as defined in the appended claims.

I claim:

1. In the manufacture of tin plate, the successive steps consisting in introducing the plates successively through a flux into and through a bath of molten tin and through an oil bath in the passage thereof out of the molten tin, subjecting the plates to roller pressure while submerged in the tin bath, to thereby smooth and flatten the coating and remove excess tin, and again subjecting the plates to roller pressure in the passage thereof through the oil bath to remove surplus tin remaining on the coated sheets, and successively feeding the plates at a uniform speed of at least 150 inches per minute into, through and out of the flux, the tin bath and the oil bath.

2. In the manufacture of tin plate, the step consisting of feeding the plates introduced into the tin pot successively into, through, and out of the flux, the tin bath and the oil bath at a uniform speed of not less than 120 inches per minute.

3. In the manufacture of tin plate, the step consisting of feeding the plates introduced into the tin pot successively into, through, and out of the flux, the tin bath and the oil bath, at a uniform speed of at least 150 inches per minute.

4. In the manufacture of tin plate, the steps consisting of introducing the plates into the tin pot, passing each plate into and through the flux into the molten tin bath and into and through the oil bath from the tin bath, squeezing the coated plate, to remove surplus molten tin therefrom, in its passage through the oil bath, and feeding each plate successively into and through and out of the flux, the tin bath and the oil bath at a substantially constant speed of not less than 120 inches per minute.

5. In the manufacture of tin plate the steps consisting of introducing the plates into the tin pot, passing each plate into and through the flux into the molten tin bath and into and through the oil bath from the tin bath, squeezing the coated plate at an intermediate point in its travel through the tin bath, to remove excess molten tin from the coated plate, again squeezing the coated plate to remove surplus molten tin therefrom in the passage of the coated plate through the oil bath, and feeding each plate successively into and through and out of the flux, the tin bath and the oil bath, at a substantially constant speed of at least 150 inches per minute.

6. In the manufacture of tin plate, the steps of successively and uninterruptedly passing each plate into and through the flux, the molten tin bath and the oil bath at one and the same uniform, relatively high rate of speed and squeezing off surplus tin from the coated plate at a single point and on the flux side of the tin bath during the travel thereof through the tin bath.

7. In the manufacture of tin plate, the steps of successively and uninterruptedly passing each plate into and through the flux, the molten tin bath and the oil bath at the same uniform, relatively high rate of speed, removing surplus tin from the coated plate at a single point and on the flux side of the tin bath during its travel through said tin bath and again removing surplus tin from the coated plate during the passage thereof through said oil bath.

In testimony whereof I have hereunto set my hand.

STEWART A. DAVIS.